

[54] HEAT TREATMENT TO DISSOLVE LOW MELTING PHASES IN SUPERALLOYS

3,272,666 9/1966 Symonds..... 148/13

[75] Inventors: James L. Walker, Schenectady; Thomas F. Sawyer, Ballston Lake, both of N.Y.

Primary Examiner—Richard O. Dean  
Attorney—Richard R. Brainard et al.

[73] Assignee: General Electric Company, Schenectady, N.Y.

[57] ABSTRACT

[22] Filed: Aug. 2, 1972

[21] Appl. No.: 277,373

**Related U.S. Application Data**

[63] Continuation of Ser. No. 100,053, Dec. 21, 1970, abandoned.

A progressive heat treatment of a superalloy is disclosed wherein the segregated low melting phases are dissolved in solid solution and diffused through the structure without melting the matrix metal and without incipiently melting any of the low melting phases. The heat treatment begins at a temperature just below that of the lowest melting constituent and finishes at a temperature below the fusion temperature of the alloy. The time of heat treatment at each successive increasing temperature is sufficient to accomplish enough diffusion to avoid melting on subsequent temperature increases, until the various phases are substantially solutionized.

[56] References Cited

**UNITED STATES PATENTS**

3,310,440 3/1967 Pearcey ..... 148/13

4 Claims, 5 Drawing Figures



PATENTED AUG 21 1973

3,753,790

SHEET 1 OF 3

Fig.1.



Fig.2.



Inventors:  
James L. Walker,  
Thomas F. Sawyer,  
by *John Austin*  
Their Attorney.

PATENTED AUG 21 1973

3,753,790

SHEET 2 OF 3

Fig. 3.



Fig. 4.



Inventors:  
James L. Walker,  
Thomas F. Sawyer,  
by *John R. Smith*  
Their Attorney.

PATENTED AUG 21 1973

3,753,790

SHEET 3 OF 3

Fig.5.



Inventors:  
James L. Walker,  
Thomas R. Sawyer,  
by *John D. Bristow*  
Their Attorney.

## HEAT TREATMENT TO DISSOLVE LOW MELTING PHASES IN SUPERALLOYS

This is a continuation, of application Ser. No. 100,053, filed Dec. 21, 1970, now abandoned.

This invention relates to superalloys and more particularly to the heat treatment of those alloys having segregated low melting phases in the as-cast condition, in order to improve their properties.

### BACKGROUND

In nickel base superalloys, of which Rene 100 and Rene 80 are typical examples, non-equilibrium phases are produced as a result of segregation during solidification. Segregates tend to form because of the non-equilibrium conditions which occur during the normal cooling of the alloy as it solidifies.

Heretofore, the alloy Rene 100 was considered as being non-solutionable. Whenever this alloy was heated above the solvus temperature in an attempt to put the different microscopic phases into solid solution, the lowest melting phase would melt. This lead to the conclusion, prevalent in the art, that within practical time limits the different low melting phases of these alloys could not be put into solid solution.

In order to improve the physical properties of an alloy, in general it is known that if the various constituents can be placed into solid solution and then precipitated out of solid solution during an "age hardening" heat treatment, the properties can be substantially improved. However, heretofore there has been no method (within practical time limits) by which alloys having substantial quantities of segregated low melting phases could be heat treated in order to place all their constituents into solid solution without incurring the problem of incipient melting.

### SUMMARY OF THE INVENTION

It is therefore an object of the present invention to provide a method for heat treating alloys having non-equilibrium segregates in order to place the segregates into solid solution.

Another object of the invention is to provide a method of improving by heat treatment, the properties of an alloy which forms low melting segregates.

Still another object of the invention is to provide a heat treated alloy body having improved physical properties.

In accordance with these and other objects of the invention, a method is provided wherein a specimen of the alloy to be heat treated is heated up to a predetermined temperature, removed and microscopically examined for incipient melting. If incipient melting has occurred, the predetermined temperature is decreased. If incipient melting had not occurred, the predetermined temperature is increased. A starting temperature for solution heat treatment is thus selected which is just below the temperature at which incipient melting of the lowest melting phase occurs. The progressive heat treatment then proceeds at increasing temperatures up to a point below the temperature at which the solid solution of the alloy melts, but proceeding at a rate sufficiently slow to accomplish enough diffusion to avoid melting the low melting phases on subsequent temperature increases, until all the low melting phases are substantially solutionized. After cooling to room temperature, the solutionizing heat treatment can then be followed by a precipitation hardening heat treatment.

### BRIEF DESCRIPTION OF THE DRAWINGS

The invention will be better understood from the following description taken in conjunction with the accompanying drawings wherein:

FIG. 1 is a photomicrograph (150 X) of a section of a Rene 100 alloy subjected to a load of 20,000 psi at a temperature of 1,800° F;

FIG. 2 is a photomicrograph (1,000 X) of Rene 100 alloy in the as-cast condition;

FIG. 3 is a photomicrograph (1,000 X) of the alloy of FIG. 2, showing the segregated area in the incipient melted condition;

FIG. 4 is a photomicrograph (1,000 X) of the same alloy Rene 100, showing the segregate partially solutionized into the surrounding alloy; and

FIG. 5 is a photomicrograph (1,000 X) of the same alloy, Rene 100, showing the alloy after the solutionizing heat treatment and air cooling.

Table I below lists the compositions of two typical known nickel base superalloys, both of which form segregated areas in the as-cast condition, similar to that illustrated in FIG. 2 of the drawings. Each of these alloys may be solution heat treated by the method according to the present invention.

Heretofore, it has not been possible to fully solutionize alloys having substantial quantities of segregated low melting phases without the occurrence of incipient melting of such phases. Therefore, the full potential strength of such alloys has heretofore not been achieved. The present invention teaches how such full solutionizing and resultant enhancing of properties can be achieved.

TABLE I

#### Nickel Base Superalloys

| Element     | Rene 80<br>Weight Percent | Rene 100<br>Weight Percent |
|-------------|---------------------------|----------------------------|
| Nickel      | Bal.                      | Bal.                       |
| 40 Chromium | 14.0                      | 9.5                        |
| Cobalt      | 9.5                       | 15.0                       |
| Titanium    | 5.0                       | 4.20                       |
| Aluminum    | 3.0                       | 5.50                       |
| Tungsten    | 4.0                       | —                          |
| Zirconium   | 0.03                      | 0.06                       |
| Molybdenum  | 4.0                       | 3.00                       |
| 45 Boron    | 0.015                     | 0.015                      |
| Silicon     | 0.2                       | 0.50                       |
| Carbon      | 0.17                      | 0.18                       |
| Manganese   | 0.2                       | 0.50                       |
| Iron        | 0.2                       | 1.0 max.                   |
| Vanadium    | —                         | 1.0                        |

It will be understood that each alloy having segregates has its own individual incipient melting temperature and that the incipient melting temperature is specific for each composition. The incipient melting temperatures for the lowest melting segregates of the alloys of Table I are as follows:

|          | °C              | °F                |
|----------|-----------------|-------------------|
| Rene 80  | 1190° to 1200°C | (2174° to 2192°F) |
| Rene 100 | 1180° to 1190°C | (2156° to 2174°F) |

The incipient melting temperatures increase as the low melting phases go into solid solution during the heat treatment.

### DISCUSSION

Among the problems of the prior art, when samples of such alloys in the as-cast condition were subjected to stress at elevated temperatures, cracks sometimes

developed. FIG. 1, for example, shows typical actual voids in the ascast Rene 100 alloy which form in the segregated zones under stress. The particular conditions of the test in Example 1, were 20,000 psi load at 1,800° F. The cracks or voids developed in these segregated areas due to the fact that these areas were the weakest zones of the alloy because they contained the low melting phases.

Accordingly, one of the aims of the present invention is to solutionize the various phases which constitute the segregated weak areas which may cause the condition illustrated in FIG. 1.

Thus, according to the present invention, the different segregates present in the as-cast body can be solutionized by gradually diffusing the segregated phases into the surrounding metal at a temperature below the incipient melting temperature. Then, after the phases of the segregate are placed into solid solution, they can be precipitated out more uniformly than they had been in the as-cast condition, to further improve the properties of the alloy. This type of heat treatment has two effects: first, it allows one to make use of essentially all of the possible precipitate which can be formed in the alloy, and secondly, it helps eliminate the areas in which the cracks or voids can form under conditions of stress at high temperature.

FIG. 2 is a photomicrograph (1,000 X) of a specimen of the Rene 100 alloy in the as-cast condition, and the segregated areas of low melting constituents are clearly visible.

#### EXAMPLE 1

To determine the starting temperature for the heat treatment, a number of specimens of nickel base alloy Rene 100 were heated at successively increasing temperatures for 10 minutes at each temperature and microscopically examined for evidence of incipient melting. Incipient melting, as illustrated in FIG. 3, was first observed in the specimen heated at 1,180° C (2,156° F). The starting temperature for the progressive heat treatment was thus determined to be 1,170° C (2,138° F). This temperature so determined was just below the incipient melting temperature for the as-cast alloy Rene 100.

The progressive heat treatment temperature was then gradually increased, and periodically specimens were removed and examined for incipient melting to make sure that diffusion without such incipient melting had taken place before the temperature was further increased. The temperature was then increased gradually to 1,220° C. During this increase, specimens were periodically removed and examined for incipient melting and to determine the progress of the solutionizing of the low melting phases. The temperature at which microscopic examination showed the the low melting phases were substantially solutionized was 1,220° C.

#### EXAMPLE 2

The procedure of Example 1 was followed for the same alloy, Rene 100, in steps to prepare samples for rupture test, but at respective holding times at each temperature. The specimens remained for convenience at the time periods listed below in Table II, which were actually longer periods than necessary because of intervening overnight and weekend circumstances.

TABLE II

|    | °C<br>1170°             | °F<br>2138°             | Time in<br>hours<br>1/4 | Remarks                                                                   |
|----|-------------------------|-------------------------|-------------------------|---------------------------------------------------------------------------|
| 5  |                         |                         |                         | Just below incipient melting temperatures of lowest melting phase         |
|    | 1180°                   | 2156°                   | 1/4                     | Gradual increase to avoid incipient melting of phases as they solutionize |
| 10 | 1190°<br>1200°          | 2174°<br>2192°          | 6 1/2<br>15 1/2         | Overnight for convenience                                                 |
| 15 | 1210°<br>1215°<br>1220° | 2210°<br>2219°<br>2228° | 7 1/2<br>1<br>64        | Weekend for convenience                                                   |
|    | Cool to about:<br>100°  |                         |                         | In inert atmosphere cooling chamber                                       |

FIG. 5 illustrates a specimen of the Rene 100 alloy which has been heat treated according to the above example 2 and subsequently cooled in an atmosphere of argon to room temperature in less than 10 minutes. The structure apparent is  $\gamma'$  phase in a matrix of  $\gamma$  phase. The  $\gamma'$  phase has precipitated out of the fully solutionized alloy during the cooling to room temperature. As compared to the as-cast alloy of FIG. 2, no low melting phases are present.

Of course, the holding times at the specific temperatures may be shorter than those listed in Table II. The minimum times at each temperature may be readily determined for the alloy being heat treated by examining a specimen periodically for incipient melting, to make sure that the temperature is not excessively increased before the segregated phases are put into solution sufficiently to increase the incipient melting point. The final temperature of the heat treatment of the Rene 100 alloy was 1,220° C (2,228° F). At this point the segregated phases were substantially all solutionized.

It will be understood, of course, that for economic reasons the length of time of the heat treatment should be as short as possible, but long enough to allow diffusion to take place without incipient melting occurring.

Thus, the progressive heat treatment according to the invention, is continued from a beginning temperature just below the incipient melting range up to a final temperature below the melting point of the alloy, at a rate and for periods of time sufficiently long at each temperature to completely diffuse the segregated elements and solutionize the low melting segregates into the balance of the alloy without incurring any incipient melting. This progressive heat treatment may be performed either by continually increasing the temperatures gradually and continuously but at a predetermined controlled rate such that the phases of the segregates are substantially solutionized; or, as in Example 2, the workpiece may be progressively subjected to increasing temperatures in a series of steps, by holding the workpiece for a specific period of time at each temperature before increasing the temperature to the next level.

The mechanical properties of the Rene 100 alloy solutionized according to the present invention were compared with an as-cast specimen of the Rene 100 alloy. The results are as follows:

#### High Temperature Static Rupture Test

(20,000 psi, 1800°F)

| Specimen                   | Hours to Rupture |
|----------------------------|------------------|
| As-cast Rene 100 alloy     | 150 hrs.         |
| Heat treated per Example 2 | 591 hrs.         |

It is thus apparent that a substantial improvement in mechanical properties can be obtained in accordance with the heat treatment of the present invention.

It will be apparent that other alloys which tend to form phases segregated capable of being solutionized can be heat treated in a manner similar to that described herein.

It will be obvious to those skilled in the art, upon reading the foregoing disclosure, that many modifications and alterations in the method steps and in the specific compositions disclosed may be made within the general context of the invention, and that numerous modifications, alterations and additions may be made thereto within the true spirit and scope of the invention as set forth in the appended claims.

What we claim as new and desire to secure by Letters Patent of the United States is:

1. A method of removing low melting segregated phases from a cast body of a nickel base superalloy which comprises the steps of:

- subjecting the cast body to a heat treatment at a temperature below the incipient melting temperature of said phases and for a sufficient time whereby the incipient melting temperature of the resulting mass is increased,
- gradually raising the temperature of the heat treatment such that the temperature is maintained below the increased incipient melting temperature

until the low melting segregated phases form a substantially homogeneous mass with the matrix, and

c. cooling said body to ambient temperature.

2. The method of claim 1, wherein said nickel base superalloy consists essentially of the following composition:

|            | Weight Percent |
|------------|----------------|
| Chromium   | 9.5            |
| Cobalt     | 15.0           |
| Titanium   | 4.20           |
| Aluminum   | 5.50           |
| Zirconium  | 0.06           |
| Molybdenum | 3.00           |
| Boron      | 0.015          |
| Silicon    | 0.50           |
| Carbon     | 0.18           |
| Manganese  | 0.50           |
| Iron       | 1.0 max        |
| Vanadium   | 1.0            |
| Nickel     | balance,       |

and the heat treatment comprises heating the cast body to a temperature of about 1,170° C. and then raising the temperature stepwise up to a maximum of 1,220° C.

3. The method according to claim 1, wherein the temperature of the heat treatment is continuously and gradually increased.

4. The method according to claim 1, wherein the temperature of the heat treatment is increased stepwise.

\* \* \* \* \*

30

35

40

45

50

55

60

65